

## UNITED STATES PATENT OFFICE.

JACOB SHOTWELL ROBESON, OF PENNINGTON, NEW JERSEY.

## COMPOSITION FOR MAKING BRIQUETTES.

No Drawing.

Application filed August 3, 1921. Serial No. 489,623.

*To all whom it may concern:*

Be it known that I, JACOB SHOTWELL ROBESON, a citizen of the United States, and resident of Pennington, in the county of 5 Mercer and State of New Jersey, have invented certain new and useful Improvements in Composition for Making Briquettes, of which the following is a specification.

10 This invention is an improvement in the manufacture of compositions of matter and includes a novel binder for use in holding together particles or masses of other material. The composition is primarily intended as a binder for the making of briquettes, and may be used in connection with coal dust or other fuel, iron ore, sand for molders' cores, or other inert material, to which it is desired to give definite form, 15 hardness and water-resistant qualities. In the manufacture of fuel briquettes it is important that the briquettes be substantially water-resistant so that little or no water be absorbed when subjected to rain or dampness during shipment or storage, and it is also important that the briquettes be not too brittle, as otherwise they break down during shipment and handling, whereby the main advantage of forming the coal dust into briquettes is lost. It is also important that the briquettes burn freely without the production of objectional volumes of smoke, and that the minimum of non-combustible products be employed.

35 In my prior Patents 841,718 and 851,381, I have disclosed a binder or adhesive compound in which sulfite cellulose liquor and wood tar are employed. Such a binder has certain advantages, but experience shows 40 that the product is too brittle for some purposes. In my prior Patent 851,380 I have disclosed a binder or adhesive compound in which sulfite cellulose liquor and molasses are employed, but if these two be employed 45 as the sole ingredients of the binder the briquette or other product, as shown by experience, would not be as water-resistant as is desirable for most purposes.

The main object of my present invention 50 is to produce a composition or adhesive material and briquette or other body employing the same, and which will be free from the objectionable qualities above referred to, and which will be inexpensive to manufacture, 55 and include only easily obtained, handled

and assembled ingredients, completely combustible and preferably of an organic nature.

In my improved adhesive composition I employ proper proportions of a sulfite solution of the non-cellulose elements of woody tissue, the liquid residue of destructive distillation preferably of woody tissue and the thick residuum of plant juices. It will be noted that all of these ingredients are of vegetable origin and include the non-cellulose ingredients in different forms. By the proper combination and proportions I avoid undue brittleness, and at the same time get water-resistant or repellent properties. In its preferred embodiment the combination 65 includes sulfite cellulose liquor, approximately 48 per cent, crude molasses, approximately 38 per cent, and wood tar, approximately 14 per cent. This binding agent may be used with coal dust or finely divided coal 70 in the proportion of about 6 per cent of the binder to 94 per cent of the coal. Other percentages of the binder may be necessary with other aggregates or material to be held in compact and definite form. When the 75 binder is used with coal dust for the making of fuel briquettes, the latter are preferably pressed in suitable molds to the proper size and shape, and are heated to approximately 80 40° Fahr. to drive off moisture and probably effect certain chemical reactions between the ingredients of the binder. The crude molasses may be that commercially sold in the market as "blackstrap" and with 85 or without previous fermentation and alcohol extraction. The sulfite cellulose liquor may be the ordinary concentrated liquor of commerce which is of approximately 30° Bé. gravity. The wood tar may be the ordinary 90 article of commerce sold under that name 95 and may be of varying degrees of plasticity.

I do not wish to be limited to the specific proportions above mentioned, as the proportions may be varied in accordance with the specific characteristics or concentration 100 of the ingredients employed. It will be noted that approximately one half of the binder is of the sulfite cellulose liquor, about one-third to two-fifths is of crude molasses, and approximately one-seventh is of wood 105 tar.

It is quite important that the tar constituent be not materially less than one seventh although a slight reduction below this amount might give satisfactory results. The 110

wood tar seems to have a very important effect in rendering the composition water-proof, and for this purpose I might use coal tar, liquid bitumens or asphalt, or mixtures of these, in place of the wood tar. All of these tarry or pitchy substances are fairly easily emulsified with sulfite cellulose liquor and the molasses.

Having thus described my invention, what I claim as new and desire to secure by Letters Patent is:—

1. A composition of matter for use as an adhesive or binding agent including sulfite solutions of the non-cellulose elements of woody tissue, liquid residue of destructive distillation of woody tissue and thick residuum of sugar bearing plant juices.

2. A binder for briquettes including molasses, sulfite cellulose liquor and wood tar.

3. A composition of matter for use as an adhesive or binding agent including sulfite cellulose liquor, approximately one-half, crude molasses, approximately two-fifths, and pitchy matter, approximately one-seventh.

4. A composition of matter for use as an adhesive or binding agent, including sulfite cellulose liquor, approximately 48 per cent, molasses, approximately 38 per cent, and tar, approximately 14 per cent.

Signed at Trenton in the county of Mercer and State of New Jersey this thirtieth day of July A. D. 1921.

JACOB SHOTWELL ROBESON.

25

30